

Nov. 9, 1954

A. DORINSON

2,694,046

LUBRICATING OIL COMPOSITION

Filed March 21, 1952



1

2,694,046

## LUBRICATING OIL COMPOSITION

Amos Dorinson, Park Forest, Ill., assignor to Sinclair Refining Company, New York, N. Y., a corporation of Maine

Application March 21, 1952, Serial No. 277,852

2 Claims. (Cl. 252—48.4)

My invention relates to a chemical additive for oils and more particularly to an additive which imparts improved lubricity and anti-seizure properties to lubricating oils thereby increasing their usefulness and value as extreme pressure lubricants and cutting oils.

It is essential that a cutting oil or extreme pressure lubricant provide adequate lubrication under conditions of both high speed and low torque and low speed and high torque. In order to impart these essential properties to lubricating oils, it is conventional to incorporate in the lubricating oils small amounts of an additive, such as sulfur-chlorinated fats and oils or sulfur-chlorinated terpene-fat mixtures. I have now found that improved anti-friction and anti-seizure properties may be imparted

specifications for No. 2 lard oil call for a maximum of 25 per cent free fatty acid content of the oil, I have thus found that superior lubricant additives may be prepared by sulfur-chlorinating a mixture of alpha-pinene and blends of commercial fatty oils of enhanced acidity, provided that the blend of commercial oil has a final free acidity as oleic acid of at least about 30 per cent.

In the preparation of a typical additive of my invention, for example, a mixture representing 100 parts by weight of alpha-pinene and 100 parts by weight of commercial oleic acid was heated to about 140° F. and 46 parts by weight of sulfur monochloride added at a rate such that the heat of reaction maintained the temperature at about 140° to 158° F. The reaction mixture was kept at about 140° F. for from about 3 to 4 hours after the completion of the addition of the sulfur monochloride and was then blown with dry air at about 122° F. to purge it of any hydrogen chloride arising from side reactions and decomposition. The mixture was next blown with air at room temperature for about 2 hours. About 0.2 per cent of propylene oxide was added to the reaction mixture to stabilize the product against further evolution of hydrogen chloride.

Other additives were prepared for test purposes using the above procedure but with various fatty substances replacing the commercial oleic acid. The various fatty substances and blends thereof and the compositions of the resulting products are indicated in Table I.

TABLE I  
Additives prepared by sulfur-chlorination of mixtures of alpha-pinene and fatty substances

| Additive No. | Starting Materials      |                                                        |                                        | Finished Additive |            |
|--------------|-------------------------|--------------------------------------------------------|----------------------------------------|-------------------|------------|
|              | Terpene                 | Fat                                                    | S <sub>2</sub> Cl <sub>2</sub> , parts | Percent S         | Percent Cl |
| I.....       | Alpha-Pinene, 100 parts | Oleic Acid, 100 parts.....                             | 46                                     | 9.07              | 10.2       |
| II.....      | do.....                 | No. 2 Lard Oil, 100 parts.....                         | 43                                     | 9.00              | 9.76       |
| III.....     | do.....                 | No. 2 Lard Oil and Oleic Acid, <sup>a</sup> 100 parts. | 45                                     | 9.69              | 9.10       |
| IV.....      | do.....                 | No. 2 Lard Oil and Oleic Acid, <sup>b</sup> 100 parts. | 45                                     | 10.00             | 9.03       |
| V.....       | do.....                 | Methyl Esters of Lard Oil, 100 parts.                  | 47                                     | 9.47              | 10.2       |

<sup>a</sup> 7.5% oleic acid and 92.5% No. 2 lard oil; final free fatty acidity of the blend 27.5%.

<sup>b</sup> 36.5% oleic acid and 63.5% No. 2 lard oil; final free fatty acidity of the blend 50%.

to lubricating oils by incorporating therein a small amount of a sulfur-chlorinated mixture of alpha-pinene and oleic acid.

The product of my invention is prepared by reacting sulfur monochloride with a mixture of alpha-pinene and oleic acid. Advantageously the mixture of alpha-pinene and oleic acid contains approximately equal parts of each substance. The improved lubricating compositions of my invention comprise lubricating oils, either solvent or acid treated, having incorporated therein about 0.5 to about 4 per cent by weight of the sulfur monochloride-alpha-pinene-oleic acid reaction product.

I have found that sulfur-chlorination of a mixture of alpha-pinene and oleic acid produces an additive unexpectedly superior, when incorporated in lubricating oils used as extreme pressure lubricants or cutting oils, to an additive obtained by sulfur-chlorinating a mixture of alpha-pinene and a neutral fat such as methyl esters of lard oil or prime lard oil. For example, I have found that at concentrations of the order of 0.5 per cent by weight of my novel additive in a heavy lubricating base oil, improved lubricity at moderate loads and superior anti-seizure properties at higher loads are realized. In addition, this superior behavior is associated with similar wear at moderate loadings and probably with not more than 5 per cent excess wear at higher loadings of that induced by sulfur chloride-pinene-neutral fat reaction product additives.

I have also found that sulfur-chlorinating a mixture of alpha-pinene and a blend of No. 2 lard oil and oleic acid yields an additive which is superior, when used in lubricants, to one prepared by sulfur-chlorinating a mixture of alpha-pinene and No. 2 lard oil. Since commercial

The commercial oleic acid used in the preparation of additives I, III and IV was a low titer, distilled red oil having an iodine value of 93.7. The No. 2 lard oil used in preparing additives II, III, and IV had a free fatty acidity as oleic acid of 21.5 per cent and an iodine value of 68.7. The free fatty acidity as oleic acid of the methyl esters of lard oil used in preparing additive V was 2.4 per cent and its iodine value was 78.9.

Evaluation of these additives was made on a Falex testing machine by the method designated as the regular or standard Falex test. In this method the load is applied in 250 pound increments and the machine is allowed to run for a full minute at each load level. Although additives may be evaluated on a Falex testing machine by the cutting oil breakdown method in which the load is increased continuously at a constant rate, a more severe test than the regular Falex method, duplicate runs tend to give more erratic results than the regular method. Since it is desirable to use the testing method with the fewest sporadic errors, the results described below are those obtained by the regular Falex procedure, the differences among the various additives being accentuated by reducing their concentrations in the oil blends.

In evaluating additives with the Falex machine it is generally accepted that the lubricity of an additive, as characterized by the slope of the curve at moderate loadings, is a different phenomenon than its anti-seizure properties, characterized by plateau-like regions in the curve. Figure 1 presents in graphical form the Falex data for 1/2 per cent solutions of additives I, II, and V, respectively, in a heavy lubricating base oil as well as data for additive I at 1/4 per cent. Gross visual inspection is sufficient to perceive the superiority of 1/2 % addi-

tive I over  $\frac{1}{2}\%$  additive V. Also,  $\frac{1}{4}\%$  additive I shows substantially the same superiority over  $\frac{1}{2}\%$  additive V up to a load of 2500 lbs., when a sudden transition, indicating the onset of incipient seizure, shifts the curve to a new torque plateau at about the same level as the plateau for  $\frac{1}{2}\%$  additive V. The curve for  $\frac{1}{2}\%$  additive II starts off better than the curve for  $\frac{1}{2}\%$  additive V (compare regions i and ii in the first-named curve with the sharp rise of region i in the second), but the sudden transitional rise to a torque of 55 lbs./ft. at 1250 lbs. load is sufficient to put  $\frac{1}{2}\%$  additive II in the same behavior class with  $\frac{1}{2}\%$  additive V at loads higher than 1000 lbs. Further, only gross visual inspection of the graph is required to demonstrate the superiority of  $\frac{1}{2}\%$  additive I over  $\frac{1}{2}\%$  additive II at loads greater than 1000 lbs. Table II summarizes the salient features of Figure 1.

TABLE II  
*Falex testing of additives*

| ADDITIVE I ( $\frac{1}{2}\%$ ) |                  |                        |                |               |
|--------------------------------|------------------|------------------------|----------------|---------------|
| Description                    | Load Range, lbs. | Torque Range, lbs. ft. | Average Torque | Average Slope |
| Plateau A.....                 | 1,500-2,250      | 28-30                  | 29             | 0.0027        |
| Plateau B.....                 | 2,750-4,000      | 37.5-40.5              | 38.5           | 0.0024        |
| Transition.....                | 2,250-2,750      | 30-37.5                | .....          | 0.015         |
| Region i.....                  | 0-250            | 0-13                   | .....          | 0.052         |
| Region ii.....                 | 250-1,000        | 13-24                  | .....          | 0.015         |
| Region iii.....                | 1,000-1,500      | 24-28                  | .....          | 0.008         |

| ADDITIVE I ( $\frac{1}{4}\%$ ) |                  |                        |                |               |
|--------------------------------|------------------|------------------------|----------------|---------------|
| Description                    | Load Range, lbs. | Torque Range, lbs. ft. | Average Torque | Average Slope |
| Plateau C.....                 | 1,750-2,500      | 30-33                  | 31.5           | 0.004         |
| Plateau D.....                 | 3,500-4,000      | 46-48                  | 47             | 0             |
| Transition (a).....            | 2,500-2,750      | 33-60                  | .....          | 0.108         |
| Transition (b).....            | 2,750-3,500      | 60-47                  | .....          | -0.017        |
| Region i.....                  | 0-250            | 0-12                   | .....          | 0.048         |
| Region ii.....                 | 250-750          | 12-20                  | .....          | 0.016         |
| Region iii.....                | 750-1,750        | 20-30                  | .....          | 0.010         |

  

| ADDITIVE II ( $\frac{1}{2}\%$ ) |                  |                        |                |               |
|---------------------------------|------------------|------------------------|----------------|---------------|
| Description                     | Load Range, lbs. | Torque Range, lbs. ft. | Average Torque | Average Slope |
| Plateau.....                    | 2,500-4,000      | 47-50                  | 48             | 0.0020        |
| Transition (a).....             | 1,000-1,250      | 25-55                  | .....          | 0.120         |
| Transition (b).....             | 1,250-1,750      | 55-40                  | .....          | -0.030        |
| Region i.....                   | 0-250            | 0-11                   | .....          | 0.044         |
| Region ii.....                  | 250-1,000        | 11-25                  | .....          | 0.019         |
| Region iii.....                 | 1,750-2,500      | 40-47                  | .....          | 0.0093        |

| ADDITIVE III ( $\frac{1}{2}\%$ ) |                  |                        |                |               |
|----------------------------------|------------------|------------------------|----------------|---------------|
| Description                      | Load Range, lbs. | Torque Range, lbs. ft. | Average Torque | Average Slope |
| Plateau.....                     | 1,750-2,750      | 37-39                  | 38             | 0.0020        |
| Transition.....                  | 1,250-1,750      | 25-37                  | .....          | 0.024         |
| Region i.....                    | 0-250            | 0-11                   | .....          | 0.044         |
| Region ii.....                   | 250-1,250        | 11-25                  | .....          | 0.014         |

| ADDITIVE IV ( $\frac{1}{2}\%$ ) |                  |                        |                |               |
|---------------------------------|------------------|------------------------|----------------|---------------|
| Description                     | Load Range, lbs. | Torque Range, lbs. ft. | Average Torque | Average Slope |
| Plateau.....                    | 1,500-2,500      | 35-38                  | 37             | 0.0030        |
| Transition.....                 | 1,250-1,500      | 30-37                  | .....          | 0.028         |
| Region i.....                   | 0-250            | 0-12                   | .....          | 0.048         |
| Region ii.....                  | 250-1,250        | 12-30                  | .....          | 0.018         |

| ADDITIVE V ( $\frac{1}{2}\%$ ) |                  |                        |                |               |
|--------------------------------|------------------|------------------------|----------------|---------------|
| Description                    | Load Range, lbs. | Torque Range, lbs. ft. | Average Torque | Average Slope |
| Plateau.....                   | 1,500-4,000      | 50-52                  | 50             | 0             |
| Transition.....                | 1,250-1,500      | 52-50                  | .....          | -0.008        |
| Region i.....                  | 0-1,250          | 0-56                   | .....          | 0.045         |

Additives I and V ( $2\%$  by weight in a heavy lubricating base oil) were further tested on the Timken machine to determine their wear characteristics at moderate pres-

5  
ures and were subjected to the two hour test on the four-ball machine to determine their wear characteristics at higher pressures. The data of Tables III and IV indicate respectively that at the moderate pressure prevailing in the Timken test there is no significant difference between the wear with the two additives and that at the higher pressures prevailing in the four ball tester the wear induced by additive I at pressures ranging from 40,000 to 150,000 pounds per square inch (the pressures prevailing in the Falex tester) is not more than about 5% in excess of that induced by additive V.

TABLE III  
*Timken testing of additives*  
2% ADDITIVE I

| Scar Width, mm. | Lever Load, lbs. | Pressure, kgm./sq. cm. |
|-----------------|------------------|------------------------|
| 1.1.....        | 22               | 715                    |
| 1.4.....        | 28               | 765                    |
| 1.5.....        | 32               | 768                    |
| 2% ADDITIVE V   |                  |                        |
| 1.1.....        | 24               | 778                    |
| 1.5.....        | 26               | 622                    |
| 1.4.....        | 32               | 812                    |

TABLE IV  
*Four-ball testing of additives*

| Load, kgm.         | Wear, cc. | Pressure, kgm./sq. cm. | Ratio * |
|--------------------|-----------|------------------------|---------|
| Base Oil b.....    | 7         | 0.0868                 | 1,400   |
| 2% Additive I..... | 7         | 0.0904                 | 1,100   |
| 2% Additive V..... | 7         | 0.0868                 | 1,400   |
| Base Oil b.....    | 20        | 0.1008                 | 22,000  |
| 2% Additive I..... | 20        | 0.1008                 | 22,000  |
| 2% Additive V..... | 20        | 0.1008                 | 22,000  |
| Base Oil b.....    | 35        | 0.1044                 | 36,100  |
| 2% Additive I..... | 35        | 0.1198                 | 24,400  |
| 2% Additive V..... | 35        | 0.1044                 | 36,100  |
| Base Oil b.....    | 60        | 0.1206                 | 46,500  |
| 2% Additive I..... | 60        | 0.1434                 | 30,000  |
| 2% Additive V..... | 60        | 0.1204                 | 49,100  |

50 \* Wear with additive divided by wear with 1095 oil.

\*\* Solvent-refined Mid-Continent oil of 100 S. U. S. at 100° F.

I claim:

1. As a composition of matter useful for the purpose of imparting lubricity and anti-seizure properties to lubricating oils, the product formed by the reaction of about 45 parts of sulfur monochloride and a mixture comprising about 100 parts of alpha-pinene and about 100 parts of oleic acid at a temperature of about 140° to 158° F.

55 2. A lubricating oil composition which comprises a mineral lubricating oil having incorporated therein about 0.5 to about 4 weight per cent of the product formed by the reaction of about 45 parts of sulfur monochloride and a mixture comprising about 100 parts of alpha-pinene and about 100 parts of oleic acid at a temperature of about 140° to 158° F.

60 References Cited in the file of this patent

UNITED STATES PATENTS

70 Number Name Date  
2,422,275 Winning et al. June 17, 1947  
2,606,182 Musselman Aug. 5, 1952